

## 1

3,335,096  
CORROSION INHIBITORS AND METHODS OF  
USING SAME  
George B. Hatch, Allison Park, Pa., assignor to  
Calgon Corporation  
No Drawing. Filed July 16, 1964, Ser. No. 383,222  
12 Claims. (Cl. 252—389)

This invention relates to new corrosion inhibiting compositions consisting essentially of sodium nitrite, sodium tetraborate, benzotriazole, and sodium silicofluoride, and mixtures thereof with sodium bicarbonate or carbonate, and to the method of inhibiting metal corrosion in closed water systems therewith.

High maintenance and replacement costs due to corrosion, deposition, valve and pump difficulties, untimely plugging of heat exchangers as well as equipment failures, have long been serious problems in closed circulating water systems, especially in view of the increasing use and complexity of closed system machinery such as diesels, internal combustion engines and high temperature hot water systems.

Sodium nitrite-sodium tetraborate-benzotriazole compositions have been used as corrosion inhibitors in essentially closed water systems for a number of years. See Liddell Patent No. 2,877,188. These compositions have given good protection for ferrous metals, copper and copper alloys, but they actually accelerate the corrosion of aluminum, lead and alloys of lead such as soft solder, i.e., lead-tin solder.

Although I am uncertain of the mechanism, I have found that the addition of sodium silicofluoride or mixtures of sodium silicofluoride and sodium bicarbonate or carbonate to a basic sodium nitrite-sodium tetraborate-benzotriazole composition substantially reduces the corrosion of aluminum, lead, and soft solder without impairing the effective corrosion inhibition of the other common metals used in closed water systems.

My invention includes compositions containing about 23-90% sodium nitrite, about 9.9-75% sodium tetraborate (calculated as the pentahydrate), about 0.1-5% ben-

## 2

zotriazole, sodium silicofluoride in about 20-34% of the amount of sodium tetraborate, and a sodium salt of carbonic acid in a quantity sufficient to supply bicarbonate ions in up to about 5% of the amount of sodium nitrite, i.e., sodium bicarbonate in up to about 5% of the amount of sodium nitrite, or sodium carbonate in up to about 3.2% of the amount of sodium nitrite, since carbonate forms bicarbonate in solution:



The preferred composition of my invention contains about 50-76% sodium nitrite, about 15-40% sodium tetraborate (calculated as the pentahydrate), 0.5-3% benzotriazole, sodium silicofluoride in about 20-34% of the amount of sodium tetraborate, and sodium bicarbonate in up to about 5% of the amount of sodium nitrite.

The following experiments with examples of the compositions of my invention demonstrate their effectiveness as metal corrosion inhibitors.

Weighed metal specimens were immersed in solutions of various corrosion inhibiting compositions dissolved in water containing 19 p.p.m. calcium, 6.0 p.p.m. magnesium (total hardness thus calculated at 77 p.p.m.  $\text{CaCO}_3$ ), 18 p.p.m. chloride, and 12 p.p.m. bicarbonate and agitated therein for five days at 35° C. After this five day exposure the metals were removed and cleaned with pickle solutions consisting of 10%  $\text{H}_2\text{SO}_4$  for admiralty, copper, and tin, 5% of 37% HCl for aluminum, 18.5% HCl and 0.1% dibutylthiourea for steel, 25% ammonium acetate for lead and soft solder, and reweighed. In order to correct for weight loss due to pickling, identical metal specimens which were not subjected to corrosion were weighed, pickled, and reweighed, and the weight loss of these blanks was subtracted from the weight loss of their respective corrosion test specimens. Using this figure as the weight loss due to corrosion, the loss of metal in milligrams per square decimeter per day was calculated.

Table I lists the concentrations and ingredients of various corrosion inhibiting compositions used in these experiments.

TABLE I

| Comp. | Conc.,<br>p.p.m. | $\text{NaNO}_2$ ,<br>percent | Benzotriazole,<br>percent | $\text{Na}_2\text{B}_4\text{O}_7 \cdot 5\text{H}_2\text{O}$ ,<br>percent | $\text{NaSiF}_6$ ,<br>percent | $\text{NaHCO}_3$ ,<br>percent | $\text{H}_3\text{BO}_3$ ,<br>percent |
|-------|------------------|------------------------------|---------------------------|--------------------------------------------------------------------------|-------------------------------|-------------------------------|--------------------------------------|
| I     | 2,000            | 74                           | 1                         | 25                                                                       |                               |                               |                                      |
| II    | 4,000            | 74                           | 1                         | 25                                                                       |                               |                               |                                      |
| III   | 2,000            | 75                           | 1                         | 4                                                                        |                               |                               |                                      |
| IV    | 2,000            | 75                           | 1                         | 3.67                                                                     |                               |                               |                                      |
| V     | 2,000            | 74                           | 1                         | 20                                                                       |                               | 2                             | 20                                   |
| VI    | 4,000            | 74                           | 1                         | 20                                                                       |                               | 5                             | 18.33                                |
| VII   | 3,000            | 49                           | 1                         | 40                                                                       |                               | 10                            |                                      |
| VIII  | 2,000            | 73                           | 2                         | 20                                                                       |                               | 5                             |                                      |
| IX    | 2,000            | 72                           | 1                         | 20                                                                       |                               | 5                             | 2                                    |
| X     | 2,000            | 71                           | 2                         | 20                                                                       |                               | 5                             | 2                                    |

Table II demonstrates the effectiveness of various examples of my invention in inhibiting corrosion under the conditions specified. It will be seen that my improved compositions (V-X) have substantially reduced the corrosion of aluminum, soft solder, and lead, without affecting the corrosion inhibition of the other metals.

5 4. A method of inhibiting corrosion of ferrous metals, copper, aluminum, lead or tin in closed water systems comprising adding to said systems the composition of claim 2 in amounts sufficient to maintain the concentration of sodium nitrite at between about 500 and about 20,000 p.p.m.

TABLE II

| Composition | Steel <sup>1</sup> | Admiralty <sup>2</sup> | Aluminum | Solder |     |     | Lead  | Tin | Copper |
|-------------|--------------------|------------------------|----------|--------|-----|-----|-------|-----|--------|
|             |                    |                        |          | A      | B   | C   |       |     |        |
| Control     | 166                | 3.9                    | 1.1      | 1.2    | 2.7 | 1.3 | 941   | 0.4 | 0.1    |
| I           | 0.2                | 0.1                    | 20.5     | 2.1    | 2.3 | 1.1 | 1,193 | 1.7 |        |
| II          |                    |                        | 6.6      |        |     |     | 50.7  |     |        |
| III         | 0.0                | 0.1                    | 3.4      | 0.2    | 1.1 | 2.8 |       |     |        |
| IV          |                    |                        |          |        |     |     |       |     |        |
| V           | 0.0                | 0.1                    | 0.6      | 0.7    | 0.9 | 0.6 | 16.3  | 2.8 |        |
| VI          | 0.1                | 0.3                    | 0.5      | 0.2    | 0.7 |     |       |     |        |
| VII         | 0.1                | 0.1                    | 0.8      |        | 0.0 |     |       |     |        |
| VIII        | 0.1                | 0.0                    | 1.0      |        |     | 1.0 | 7.3   |     | 0.0    |
| IX          |                    |                        | 0.4      |        |     |     | 0.7   | 0.4 |        |
| X           | 0.2                | 0.0                    | 0.8      |        |     |     | 0.5   | 1.6 | 0.0    |

<sup>1</sup> AISI-SAE 1010. <sup>2</sup> ASTM B171.

Solder A is 50% lead, 50% tin; Solder B is 60% lead, 40% tin; Solder C is 70% lead, 30% tin; all figures given as metal loss in milligrams per square decimeter per day, many being averages of numerous tests. The control was carried out under identical conditions, but no corrosion inhibitor was added.

The compositions of my invention may be added to closed water systems in sufficient amounts to maintain the concentration of sodium nitrite at from about 500 to about 20,000 p.p.m., but it is most economical to maintain the sodium nitrite concentration at 1000-3000 p.p.m.

The pH range in the water system may be maintained from about 7 to about 9, but it is preferable to have a pH of about 8-8.5 and to obtain this pH by regulating the relative amounts of sodium tetraborate and sodium silicofluoride.

Thus, my invention relates to improved corrosion inhibiting compositions consisting essentially of sodium nitrite, sodium tetraborate, benzotriazole, sodium silicofluoride, and mixtures thereof with sodium bicarbonate or carbonate, and to the method of inhibiting the corrosion of metals in closed water systems therewith.

I do not intend to be limited to the specific compositions disclosed herein for illustrative purposes. My invention may be otherwise practiced and embodied within the scope of the following claims.

I claim:

1. A composition for inhibiting corrosion of ferrous metals, copper, aluminum, lead or tin in closed water systems consisting essentially of about 23-90% sodium nitrite, about 9.9-75% sodium tetraborate (calculated as the pentahydrate), about 0.1-5% benzotriazole, sodium silicofluoride at about 20-34% of the amount of sodium tetraborate, and a sodium salt of carbonic acid in a quantity sufficient to supply bicarbonate ions in up to about 5% of the amount of sodium nitrite.

2. A composition for inhibiting corrosion of ferrous metals, copper, aluminum, lead or tin in closed water systems consisting essentially of about 50-76% sodium nitrite, about 15-40% sodium tetraborate (calculated as the pentahydrate), about 0.5-3% benzotriazole, sodium silicofluoride at about 20-34% of the amount of sodium tetraborate, and a sodium salt of carbonic acid in a quantity sufficient to supply bicarbonate ions in up to about 5% of the amount of sodium nitrite.

3. A method of inhibiting corrosion of ferrous metals, copper, aluminum, lead or tin in closed water systems comprising adding to said systems the composition of claim 1 in amounts sufficient to maintain the concentration of sodium nitrite at between about 500 and about 20,000 p.p.m.

25 5. A method of inhibiting corrosion of ferrous metals, copper, aluminum, lead or tin in closed water systems comprising adding to said systems the composition of claim 1 in amounts sufficient to maintain the concentration of sodium nitrite at between about 500 and about 30 20,000 p.p.m., the amount of sodium tetraborate and sodium silicofluoride in said composition being such as to obtain a pH in the system of between about 8.0 and about 8.5.

35 6. A method of inhibiting corrosion of ferrous metals, copper, aluminum, lead or tin in closed water systems comprising adding to said systems the composition of claim 2 in amounts sufficient to maintain the concentration of sodium nitrite at between about 500 and about 40 20,000 p.p.m., the amount of sodium tetraborate and sodium silicofluoride in said composition being such as to obtain a pH in the system of between about 8.0 and 8.5.

45 7. A method of inhibiting corrosion of ferrous metals, copper, aluminum, lead or tin in closed water systems comprising adding to said systems the composition of claim 1 in amounts sufficient to maintain the concentration of sodium nitrite at between about 1,000 and about 3,000 p.p.m.

50 8. A method of inhibiting corrosion of ferrous metals, copper, aluminum, lead or tin in closed water systems comprising adding to said systems the composition of claim 2 in amounts sufficient to maintain the concentration of sodium nitrite at between about 1,000 and about 3,000 p.p.m.

55 9. A method of inhibiting corrosion of ferrous metals, copper, aluminum, lead or tin in closed water systems comprising adding to said systems the composition of claim 1 in amounts sufficient to maintain the concentration of sodium nitrite at between about 1,000 and about 60 3,000 p.p.m., the amount of sodium tetraborate and sodium silicofluoride in said composition being such as to obtain a pH in the system of between about 8.0 and about 8.5.

65 10. A method of inhibiting corrosion of ferrous metals, copper, aluminum, lead or tin in closed water systems comprising adding to said systems the composition of claim 2 in amounts sufficient to maintain the concentration of sodium nitrite at between about 1,000 and about 3,000 p.p.m., the amount of sodium tetraborate and sodium silicofluoride in said composition being such as to obtain a pH in the system of between about 8.0 and 8.5.

70 11. A method of inhibiting corrosion of ferrous metals, copper, aluminum, lead or tin in closed water systems comprising adding to said systems the composition of claim 1 in amounts sufficient to maintain the concentra-

tion of sodium nitrite at between about 500 and about 20,000 p.p.m., and maintaining a pH in said systems of between about 7 and about 9.

12. A method of inhibiting corrosion of ferrous metals, copper, aluminum, lead or tin in closed water systems comprising adding to said systems the composition of claim 2 in amounts sufficient to maintain the concentration of sodium nitrite at between about 500 and about 20,000 p.p.m., and maintaining a pH in said systems of between about 7 and about 9.

**References Cited****UNITED STATES PATENTS**

|           |        |           |         |
|-----------|--------|-----------|---------|
| 2,795,560 | 6/1957 | Williams  | 252—387 |
| 2,877,188 | 3/1959 | Liddell   | 252—389 |
| 3,024,099 | 3/1962 | Martinson | 252—387 |

LEON D. ROSDOL, *Primary Examiner.*

SAMUEL H. BLECH, *Examiner.*

10 M. WEINBLATT, *Assistant Examiner.*